

Dec. 16, 1969

FUMIHIKO NISHIO ET AL

3,484,242

SILVER HALIDE EMULSIONS STABILIZED WITH COMPOUNDS  
HAVING A SINGLE AZIRIDINE GROUP IN THE MOLECULE

Filed April 12, 1965



INVENTORS  
FUMIHIKO NISHIO  
NOBUO YAMAMOTO  
MITSUNORI SUGIYAMA  
JUN HAYASHI

BY

Buckman and Archer  
ATTORNEYS

1

3,484,242

## SILVER HALIDE EMULSIONS STABILIZED WITH COMPOUNDS HAVING A SINGLE AZIRIDINE GROUP IN THE MOLECULE

Fumihiro Nishio, 450 Yatsu, Odawara-shi; Mitsunori Sugiyama, 677 Mukouhara, Yamakita-machi, Ashigarakami-gun; Nobuo Yamamoto, 538 Mukaidi, Minamiasigara-machi, Ashigarakami-gun; Jun Hayashi, 932 Kano Minamishigara-machi, Ashigarakami-gun, all of Kanagawa-ken, Japan

Filed Apr. 12, 1965, Ser. No. 447,344

Claims priority, application Japan, Apr. 17, 1964,  
39/21,483

Int. Cl. G03c 1/34

U.S. Cl. 96—109

10 Claims

5

2

An example of such compounds is a compound shown by the following general formula



wherein X represents —CO—, —CS—, or —SO<sub>2</sub>—; Y represents an alkyl group, an aryl group, or



(where R<sub>4</sub> and R<sub>5</sub> each represents hydrogen, an alkyl group, a cyclic alkyl group, an aryl group, or an aralkyl group); and R<sub>1</sub>, R<sub>2</sub> and R<sub>3</sub> each represents a hydrogen atom, a methyl group, or an ethyl group.

Specific examples of compounds shown by the above-mentioned formula are

25



30



35



40



45



50



55



60



65



70



75



80



wherein R<sub>1</sub>, R<sub>2</sub> and R<sub>3</sub> are each hydrogen, a methyl group or an ethyl group.

The present invention relates to a silver halide photographic material containing a fogging inhibitor and a stabilizer.

It has been well known that the photographic sensitivity of a silver halide photographic emulsion can be very effectively increased by the addition of natural active gelatin, a compound containing unstable sulfur, a noble metal salt, a polyalkylene oxide derivative, and the like. However, since fogging tends to be increased by the addition of such materials, the addition of a fogging inhibitor is necessary to suppress the increase of fogging.

Many fogging inhibitors were reported for suppressing such fogging but though the addition of these compounds decreases fogging of a photographic material, it reduces the sensitivity of the photographic material.

Therefore, an object of this invention is to provide a fogging inhibitor for a silver halide photographic material that does not reduce the sensitivity of the photographic material.

Another object of this invention is to provide a silver halide photographic emulsion the fogging of which is suppressed without reducing its sensitivity.

A further object of this invention is to provide a process for suppressing the formation of fog in a photographic material when it is preserved under severe conditions of high temperature and high humidity.

An additional object of this invention is to provide a photographic emulsion, the sensitivity and the contrast of which are scarcely affected by aging.

A still further object of this invention is to provide a process for suppressing the formation of fog without decreasing the sensitivity of a photographic material in cases where a gelatin coating of the photographic material is preliminary hardened with formalin, etc., prior to its development.

These objects can be attained in the present invention by the addition of a compound having a single aziridine group. Typical examples of compounds having a single aziridine group in the molecule are shown below.



and



Other types of the compound used as an antifogging agent in this invention is a compound shown by the general formula



20  
25

(II)

wherein A represents H,  $C_1-C_4$  alkyl,  $-COOR_7$  (wherein  $R_7$  is an alkyl group, an aryl group, or an aralkyl group),  $-CN$ ,  $-CONH_2$ ,  $-OCHC_3$ , or an aryl group;  $R_1$ ,  $R_2$ , and  $R_3$  each represents a hydrogen atom, a methyl group, or an ethyl group;  $R_6$  represents a hydrogen atom, a methyl group, or  $-CH_2COOR_8$  (where  $R_8$  is an alkyl group); and  $m$  and  $n$  each represents 0 or 1.

Specific examples of the compound shown by Formula II are



A further type of antifogging compound used in this invention is one shown by the general formula



(III)

wherein  $R_1$ ,  $R_2$ , and  $R_3$  each represents a hydrogen atom, a methyl group, or an ethyl group and  $Z_1$  and  $Z_2$  each represents  $-NH_2$ ,  $-NH.R_4$ ,



30 or  $O-R_4$  (where  $R_4$  and  $R_5$  each represents a hydrogen atom, an alkyl group, a cyclic alkyl group, an aryl group, or an aralkyl group).

Specific examples of compounds shown by Formula III are



70

75

(33)



(34)



(35)



(36)



The above-illustrated compounds each having one aziridine group in the molecule may be prepared by the addition reaction of an isocyanate or an active vinyl compound with ethyleneimine or an alkyl ethyleneimine (cf., Annalen der Chemie; vol. 556, page 210) or the substitution reaction of an active halogen compound with ethyleneimine or an alkyl ethyleneimine (cf., Berichte der Chemie; vol. 32, page 2037 and J. of American Chemical Society; vol. 77, page 5918).

The compounds used in this invention each having one aziridine group



(wherein R<sub>1</sub>, R<sub>2</sub>, and R<sub>3</sub> each represents a hydrogen atom, an ethyl group or a methyl group) in the molecule may be used alone or as a mixture thereof. Further, they may be used with other stabilizers.

The fogging inhibitor of this invention may be added in an emulsion at any time before the emulsion is applied on the support, but it is preferably added at a time between after-ripening and coating. There is no limit on the amount of the compound, but a suitable amount is 0.1-100 g. per mole of AgX (where X represents a halogen atom) in the silver halide photographic emulsion.

In the above explanation, the fogging inhibitor of this invention is described as being added to a silver halide

photographic emulsion, but the invention is not so limited, since the compound may also be added to a protective coating layer of the photographic material. In the latter case, a suitable amount of the compound is 0.5-500 g. per 1 kg. in gelatin of the protective coating layer.

5 The fogging inhibitor of this invention may suitably be incorporated in the photographic sensitive emulsion and/or protective coating in the form of a solution in a solvent having no bad effect on the silver halide photographic emulsion, such as water, a lower alcohol (e.g., methyl alcohol, ethyl alcohol, or isopropyl alcohol), or a ketone (e.g., acetone).

10 The fogging inhibitor of this invention can be incorporated into such photographic materials as, a negative emulsion for black and white photography, an X-ray emulsion, a coupler-in-emulsion type color photographic emulsion wherein a color coupler is incorporated in the emulsion, and a coupler-in-developer type color photographic emulsion wherein a color coupler is incorporated 20 in a developer. However, the best results are obtained in the case a silver iodobromide gelatin emulsion.

15 The silver halide photographic emulsion may be sensitized chemically by a conventional method, such as, by the addition of a compound containing an unstable sulfur, e.g., ammonium thiosulfate or an aryl thiourea (cf. P. Glafkides Chimie Photographique 2 em Edition, Publication Photocinema, Paul Montel Paris; page 297-299, 1957), by the addition of a gold compound, e.g. a complex salt of monovalent gold and thiocyanic acid (cf. ibid.; page 301), by the addition of a polyalkylene oxide derivative, or by a mixture thereof. Further, the silver halide photographic emulsion may be optically sensitized by the addition of an optical sensitizer such as a cyanine dye or a merocyanine dye (cf., Shinichi Kikuchi, "Kagaku Shashin Binran" (the 2nd volume), page 13-24, 1959 published by Maruzen Co.).

20 The invention will be explained further by the following examples referring to the accompanying drawing showing the relation between exposure and density of 40 color film (No. 1) that did not contain the fogging inhibitor of this invention and color film (No. 2 to No. 5) containing a fogging inhibitor of this invention.

#### EXAMPLE 1

45 A sulfur-sensitized and gold-sensitized high speed gelatin-silver iodobromide negative emulsion to which was added methyl-3-(1-aziridinyl)-propionate (Compound 16) or 1-(2-methyl-1-aziridinyl)-propionamide (Compound 19), was coated on a film base. The prepared sensitive 50 film was exposed on a sensitometer NSG Type-II (made by Tokyo Shibaura Electric Co.) and then developed for 8 minutes at 20° C. in a developer having the following composition:

|    |                                |       |       |     |
|----|--------------------------------|-------|-------|-----|
| 55 | N-methyl-p-aminophenol sulfate | ----- | g     | 2   |
|    | Sodium sulfite (anhydrous)     | ----- | g     | 100 |
|    | Hydroquinone                   | ----- | g     | 5   |
|    | Borax                          | ----- | g     | 2   |
|    | Water to                       | ----- | liter | 1   |

60 The photographic properties of the developed photographic film were determined and compared with those of a photographic film prepared and developed under the same conditions except that the fogging inhibitor of this invention was not used. The results were as follows:

| Name of compound | Quantity<br>(g./l. mol of<br>AgX) | Relative<br>sensitivity | Fog  |             |
|------------------|-----------------------------------|-------------------------|------|-------------|
|                  |                                   |                         | None | Compound 16 |
| None             | -----                             | 100                     | 100  | 0.14        |
| Compound 16      | 7.6                               | 100                     | 100  | 0.12        |
| Do               | 15.2                              | 97                      | 97   | 0.10        |
| Compound 19      | 15.0                              | 98                      | 98   | 0.11        |
| Do               | 30.0                              | 92                      | 92   | 0.09        |

As shown in the above results, the formation of fog was clearly suppressed by the fogging inhibitor of this invention.

7  
EXAMPLE 2

A sulfur-sensitized and gold-sensitized highly sensitive gelatin-silver iodobromide X-ray emulsion, to which was added N,N-ethylene-N'-phenyl urea (Compound 4) or 1-aziridinyl-propionitrile (Compound 18), was coated on a film base. The prepared photographic film was exposed on a sensitometer NSG Type-II and then developed for 6 minutes at 20° C. in a developer having the following composition.

|                                |         |    |
|--------------------------------|---------|----|
| N-methyl-p-aminophenol sulfate | g--     | 2  |
| Sodium sulfite (anhydrous)     | g--     | 80 |
| Hydroquinone                   | g--     | 8  |
| Sodium carbonate (anhydrous)   | g--     | 40 |
| Potassium bromide              | g--     | 3  |
| Water to                       | liter-- | 1  |

The photographic properties of the thus developed photographic film were compared with those of a photographic film treated under the same conditions except that the fogging inhibitor of this invention was not used. The results are shown below, which showed that the formation of fog was clearly suppressed by the addition of the fogging inhibitor of this invention.

| Name of compound | Quantity<br>(g./l. mol of<br>AgX) | Relative<br>sensitivity | Fog  |
|------------------|-----------------------------------|-------------------------|------|
| None             | -----                             | 100                     | 0.19 |
| Compound 4       | 4.1                               | 97                      | 0.16 |
| Do               | 8.2                               | 94                      | 0.11 |
| Compound 18      | 11.5                              | 97                      | 0.13 |
| Do               | 23.0                              | 92                      | 0.17 |

## EXAMPLE 3

A sulfur- and gold-sensitized gelatin-silver iodobromide reversal color emulsion, to which was added 1-acetyl-2-methyl-aziridine (Compound 12), methyl - 3 - (1-aziridinyl)-propionate (Compound 16), or 2 - (1 - aziridinyl)-4,6-bis - methoxy - 1,3,5 - triazine (Compound 28), was coated on a film base. The sensitive film was exposed on a sensitometer NSG Type-II, treated in a hardening bath having the following composition for 3 minutes at 27° C.

|                      |         |    |
|----------------------|---------|----|
| Sodium pyrophosphate | g--     | 20 |
| Sodium sulfate       | g--     | 50 |
| 37 formaldehyde      | ml--    | 17 |
| 10% caustic soda     | ml--    | 1  |
| Water to             | liter-- | 1  |

rinsed with water for 4 minutes at 27° C., and then developed for 7 minutes at 27° C. in a developer having the following composition:

|                                |         |     |
|--------------------------------|---------|-----|
| N-methyl-p-aminophenol sulfate | g--     | 1   |
| Hydroquinone                   | g--     | 10  |
| Sodium sulfite (anhydrous)     | g--     | 60  |
| Potassium bromide              | g--     | 5   |
| Potassium thiocyanate          | g--     | 1.5 |
| 0.1% potassium iodide          | ml--    | 5   |
| Caustic soda                   | g--     | 2   |
| Water to                       | liter-- | 1   |

The photographic properties of the thus developed photographic film were compared with those of a photographic film prepared and treated under the same conditions except that the fogging inhibitor of this invention was not added and the results were as follows. This showed that the formation of fog was effectively suppressed without reducing the sensitivity by the addition of the fogging inhibitor.

| Compound    | Quantity<br>(g./l. mol of<br>AgX) | Relative<br>sensitivity | Fog  |
|-------------|-----------------------------------|-------------------------|------|
| None        | -----                             | 100                     | 0.85 |
| Compound 12 | 5.95                              | 112                     | 0.52 |
| Do          | 11.9                              | 108                     | 0.31 |
| Compound 16 | 7.6                               | 130                     | 0.36 |
| Do          | 15.2                              | 115                     | 0.24 |
| Compound 28 | 5.46                              | 130                     | 0.32 |
| Do          | 10.92                             | 120                     | 0.12 |

8  
EXAMPLE 4

1 - benzoyl - aziridine (Compound 13) or 2 - (1-aziridinyl)-4-anilino-6-phenoxy-1,3,5-triazine (Compound 34) was added to a 5% gelatin solution and 5 ml. of the solution was applied on a cabinet size dry plate (about 200 sq. cm.) that had been coated with a sulfur- and gold-sensitized gelatin-silver iodobromide emulsion for reversal color photographic material. The double-coated dry plate was exposed on a sensitometer NSG Type-II and then developed in a developer having the following composition for 7 minutes at 27° C.

|                                |         |     |
|--------------------------------|---------|-----|
| N-methyl-p-aminophenol sulfate | g--     | 1   |
| Sodium sulfite (anhydrous)     | g--     | 60  |
| Hydroquinone                   | g--     | 10  |
| Potassium bromide              | g--     | 5   |
| Potassium thiocyanate          | g--     | 1.5 |
| 0.1% potassium iodide          | ml--    | 5   |
| Caustic soda                   | g--     | 2   |
| Water to                       | liter-- | 1   |

The photographic material of this example was compared with the same photographic material that did not include the fogging inhibitor of this invention but where all other conditions were the same. The results are shown in the following table, which showed that fogging formation was remarkably suppressed.

| Compound    | (mg./5 ml. of<br>5% gelatin) | Relative<br>sensitivity | Fog  |
|-------------|------------------------------|-------------------------|------|
| None        | -----                        | 100                     | 0.18 |
| Compound 13 | 0.5                          | 98                      | 0.16 |
| Do          | 1.0                          | 94                      | 0.13 |
| Compound 34 | 21.0                         | 96                      | 0.11 |
| Do          | 42.0                         | 91                      | 0.08 |

## EXAMPLE 5

1 - (p - tolsulfonyl) - aziridine (Compound 15) or 1-phenethyl-aziridine (Compound 27) was added to a 5% gelatin solution and 5 ml. of the solution was applied on a cabinet size dry plate (about 200 sq. cm.) that had been coated with a sulfur- and gold-sensitized gelatin-silver iodobromide emulsion for reversal color photographic material.

The double-coated dry plate was exposed, hardened, rinsed with water, and then developed as in Example 3, and was compared to the same photographic material treated under the same conditions without the addition of the fogging inhibitor of this invention. The results are shown in the following table, which showed the fogging formation was remarkably suppressed.

| Compound    | Quantity<br>(mg./5 ml. of<br>5% gelatin) | Relative<br>sensitivity | Fog  |
|-------------|------------------------------------------|-------------------------|------|
| None        | -----                                    | 100                     | 0.76 |
| Compound 15 | 0.5                                      | 110                     | 0.32 |
| Do          | 1.0                                      | 120                     | 0.19 |
| Compound 27 | 19.0                                     | 115                     | 0.29 |
| Do          | 38.0                                     | 126                     | 0.16 |

## EXAMPLE 6

A sulfur- and gold-sensitized gelatin-silver iodobromide emulsion for reversal color photographic material, to which was added with N,N-ethylene-N'-cyclohexyl urea (Compound 3) or 2-(1-aziridinyl)-4,6-bis-ethylamino-1,3,5-triazine (Compound 31), was applied on a film base. The sensitive film was exposed and treated as follows:

|                              | (° C.) | (min.) |
|------------------------------|--------|--------|
| 1. Pre-hardening             | 27     | 3      |
| 2. Water rinsing             | 27     | 4      |
| 3. Negative development      | 27     | 7      |
| 4. Water rinsing             | 27     | 2      |
| 5. Reversal flash exposure   | 27     | -----  |
| 6. Color development         | 27     | 5      |
| 7. Water rinsing             | 27     | 1      |
| 8. Silver bleaching          | 27     | 5      |
| 9. Fixing                    | 27     | 3      |
| 10. Water rinsing and drying | 27     | -----  |

The compositions of the above treating baths were as follows:

- (1) Pre-hardening bath: same as described in Example 3.
- (2) Negative developing solution: same as described in Example 3.

- (3) Color developing solution:

|                                                     |       |      |
|-----------------------------------------------------|-------|------|
| Sodium sulfite                                      | g.    | 5.0  |
| N,N'-diethyl paraphenylenediamine hydrochloride     | g.    | 1.2  |
| Sodium carbonate (monohydrate)                      | g.    | 20.0 |
| Potassium bromide                                   | g.    | 0.3  |
| 0.1% potassium iodide                               | ml.   | 2.0  |
| 4-(Paratoluene sulfonamide)-omega-benzoyl acetamide | g.    | 1.0  |
| Caustic soda                                        | g.    | 4.0  |
| Water to                                            | liter | 1    |

- (4) Silver bleaching solution:

|                        |       |    |
|------------------------|-------|----|
| Potassium ferricyanide | g.    | 60 |
| Potassium bromide      | g.    | 20 |
| Water to               | liter | 1  |

- (5) Fixing solution:

|                    |    |     |
|--------------------|----|-----|
| Sodium thiosulfate | g. | 100 |
| Sodium sulfite     | g. | 15  |

The film was then bleached and fixed to remove undeveloped silver halide and reduced silver using a bleaching solution and a fixing solution having the following compositions respectively:

5 Bleaching solution:

|                        |       |     |
|------------------------|-------|-----|
| Potassium ferricyanide | g.    | 100 |
| Potassium bromide      | g.    | 20  |
| Water to               | liter | 1   |

Fixing solution:

|                            |       |     |
|----------------------------|-------|-----|
| Sodium thiosulfate         | g.    | 200 |
| Sodium sulfite (anhydrous) | g.    | 20  |
| 28% Acetic acid            | g.    | 45  |
| Boric acid                 | g.    | 7.5 |
| Potassium alum             | g.    | 20  |
| Water to                   | liter | 1   |

After treating, the density was measured using a green filter. The obtained results were compared with those of a film where a photographic material prepared under the same conditions but without having the fogging inhibitor of this invention was treated under the same conditions. The results are shown in the following table.

| Compound    | Quantity (g./l. mol AgX) | Fresh Magenta colored fog | Fresh Magenta relative sensitivity | Magenta <sup>1</sup> colored fog | Magenta <sup>1</sup> relative sens. |
|-------------|--------------------------|---------------------------|------------------------------------|----------------------------------|-------------------------------------|
| None        |                          | 0.21                      | 100                                | 0.26                             | 100                                 |
| Compound 4  | 3.52                     | 0.16                      | 97                                 | 0.14                             | 103                                 |
| Do          | 7.04                     | 0.15                      | 95                                 | 0.09                             | 97                                  |
| Do          | 10.56                    | 0.12                      | 93                                 | 0.09                             | 97                                  |
| Do          | 14.08                    | 0.11                      | 91                                 | 0.07                             | 97                                  |
| Compound 28 | 8.80                     | 0.16                      | 100                                | 0.08                             | 99                                  |
| Do          | 17.60                    | 0.16                      | 95                                 | 0.09                             | 90                                  |
| Do          | 26.40                    | 0.12                      | 98                                 | 0.07                             | 90                                  |

<sup>1</sup> After aging for 2 days at 50° C. and 80% R.H.

The photographic properties of the thus obtained color photographic film were compared with those of a film treated under the same conditions but containing no fogging inhibitor of this invention. The results are shown in the following table, which show that the maximum density after color development was remarkably increased caused by the reduction of fogging in the negative development.

| Compound    | Quantity (g./l. mole of AgX) | Max. density | Characteristic curve <sup>1</sup> |
|-------------|------------------------------|--------------|-----------------------------------|
| None        |                              | 2.0          | No. 1                             |
| Compound 3  | 13.0                         | 2.3          | No. 2                             |
| Do          | 26.0                         | 3.0          | No. 3                             |
| Compound 31 | 7.3                          | 2.2          | No. 4                             |
| Do          | 14.6                         | 2.7          | No. 5                             |

<sup>1</sup> These curves are shown in the accompanying drawing.

### EXAMPLE 7

A sulfur- and gold-sensitized gelatin-silver iodobromide emulsion for a negative color photographic material was mixed with 1-(3-sulfo-4-phenoxy)benzene-3-heptadecyl-5-pyrazolone as a coupler by adding 20 parts by weight of an aqueous alkaline solution of the coupler (the coupler 1 g. per 2.5 ml. of 5% caustic soda) per 100 parts by weight of the emulsion, and the mixture was added to N,N-ethylene-N'-phenyl urea (Compound 4) or 2-(1-aziridinyl)-4,6-bismethoxy-1,3,5-triazine (Compound 28). The emulsion was, after adjusting the pH to 7.0 with citric acid, applied on a film base. The obtained sensitive film was subjected to a conventional color development using a color developing solution having the following composition:

|                                      |       |      |
|--------------------------------------|-------|------|
| N,N-diethyl paraaminoaniline sulfate | g.    | 2.0  |
| Sodium sulfite                       | g.    | 2.0  |
| Sodium carbonate (monohydrate)       | g.    | 50.0 |
| Hydroxylamine hydrochloride          | g.    | 1.5  |
| Potassium bromide                    | g.    | 1.0  |
| Water to                             | liter | 1    |

From the above table it is clear that the magenta colored fog was markedly reduced while the sensitivity was not much reduced. Moreover, it should be noticed that the photographic material of this invention was stable after aging.

Almost the same results were obtained with other compounds having a single aziridine group.

What is claimed is:

1. A photographic material comprising a support, and a silver halide photographic emulsion layer containing a stabilizing amount as a fogging inhibitor, said fogging inhibitor being a compound selected from the group consisting of:



wherein X represents a member selected from the class consisting of  $-CO-$ ,  $-CS-$ , and  $-SO_2-$ ; Y represents

a member selected from the class consisting of an alkyl group, an aryl group, and



R<sub>4</sub> and R<sub>5</sub> each represents a member selected from the class consisting of a hydrogen atom, an alkyl group, a cyclic alkyl group, an aryl group, and an aralkyl group; R<sub>1</sub>, R<sub>2</sub>, and R<sub>3</sub> each represents a member selected from the class consisting of a hydrogen atom, a methyl group, and an ethyl group; A represents a member selected from the class consisting of a hydrogen atom, C<sub>1</sub>-C<sub>4</sub> alkyl, —COOR<sub>7</sub> (where R<sub>7</sub> represents a member selected from the class consisting of an alkyl group, an aryl group, and an aralkyl group), —CN, —CONH<sub>2</sub>, COCH<sub>3</sub>, and an aryl group; R<sub>6</sub> represents a member selected from the class consisting of a hydrogen atom, a methyl group, and —CH<sub>2</sub>COOR<sub>8</sub>;

R<sub>8</sub> represents an alkyl group; m and n each represents 0 or 1; and Z<sub>1</sub> and Z<sub>2</sub> each represents a member selected from the class consisting of —NH<sub>2</sub>, —NH.R<sub>4</sub>,



and —O—R<sub>4</sub> (where R<sub>4</sub> and R<sub>5</sub> are as defined above).

2. The silver halide photographic sensitive material as claimed in claim 1 wherein the amount of said compound is about 0.1 to 100 g. per 1 mol of the silver halide in said emulsion.

3. The silver halide photographic sensitive material as claimed in claim 1 wherein said compound is one shown by the general formula



wherein X represents a member selected from the class consisting of —CO—, —CS—, and —SO<sub>2</sub>—; Y represents a member selected from the class consisting of an alkyl group, an aryl group, and



(where R<sub>4</sub> and R<sub>5</sub> each represents a member selected from the class consisting of a hydrogen atom, an alkyl group, a cyclic alkyl group, an aryl group, and an aralkyl group); and R<sub>1</sub>, R<sub>2</sub>, and R<sub>3</sub> each represents a hydrogen atom, a methyl group, and an ethyl group.

4. The silver halide photographic sensitive material as claimed in claim 1 wherein said compound is one shown by the general formula



wherein A represents a member selected from the class consisting of a hydrogen atom, C<sub>1</sub>-C<sub>4</sub> alkyl, —COOR<sub>7</sub> (where R<sub>7</sub> represents a member selected from the class consisting of an alkyl group, an aryl group, and an aralkyl group), —CN, —CONH<sub>2</sub>, COCH<sub>3</sub>, and an aryl group; R<sub>1</sub>, R<sub>2</sub>, and R<sub>3</sub> each represents a member selected from the class consisting of a hydrogen atom, a methyl group, and an ethyl group; R<sub>6</sub> represents a member selected from the class consisting of a hydrogen atom, a methyl group, and —CH<sub>2</sub>COOR<sub>8</sub> (where R<sub>8</sub> represents an alkyl group); and m and n each represents 0 or 1.

5. The silver halide photographic sensitive material as claimed in claim 1 wherein said compound is one shown by the general formula



wherein R<sub>1</sub>, R<sub>2</sub>, and R<sub>3</sub> each represents a member selected from the class consisting of a hydrogen atom, a methyl group, and an ethyl group and Z<sub>1</sub> and Z<sub>2</sub> each represents a member selected from the class consisting of —NH<sub>2</sub>, —NH.R<sub>4</sub>,



and —O—R<sub>4</sub> (where R<sub>4</sub> and R<sub>5</sub> each represents a member selected from the class consisting of a hydrogen atom, an alkyl group, a cyclic alkyl group, an aryl group, and an aralkyl group).

6. A silver halide photographic sensitive material comprising a support, a silver halide photographic emulsion layer, and a protective coating layer, at least one of said layers containing a stabilizing amount of a fogging inhibitor, said fogging inhibitor being a compound selected from the group consisting of:



and



wherein X represents a member selected from the class consisting of —CO—, —CS—, and —SO<sub>2</sub>—; Y represents a member selected from the class consisting of an alkyl group, an aryl group, and



R<sub>4</sub> and R<sub>5</sub> each represents a member selected from the class consisting of a hydrogen atom, an alkyl group, a cyclic alkyl group, an aryl group, and an aralkyl group; R<sub>1</sub>, R<sub>2</sub>, and R<sub>3</sub> each represents a member selected from the class consisting of a hydrogen atom, a methyl group, and an ethyl group; A represents a member selected from the class consisting of a hydrogen atom, C<sub>1</sub>-C<sub>4</sub> alkyl, —COOR<sub>7</sub> (where R<sub>7</sub> represents a member selected from the class consisting of an alkyl group, an aryl group, and an aralkyl group), —CN, —CONH<sub>2</sub>, COCH<sub>3</sub>, and an aryl group; R<sub>6</sub> represents a member selected from the class consisting of a hydrogen atom, a methyl group, and —CH<sub>2</sub>COOR<sub>8</sub>; R<sub>8</sub> represents an alkyl group; m and n each represents 0 or 1; and Z<sub>1</sub> and Z<sub>2</sub> each represents a member selected from the class consisting of —NH<sub>2</sub>, —NH.R<sub>4</sub>,



and —O—R<sub>4</sub> (where R<sub>4</sub> and R<sub>5</sub> are as defined above).

## 13

7. The silver halide photographic sensitive material as claimed in claim 6 wherein said layer containing the compound is the silver halide photographic emulsion layer and the amount of said compound is about 0.1-100 g. per 1 mole of the silver halide in said emulsion.

8. The silver halide photographic sensitive material as claimed in claim 6 wherein said layer containing the compound is a protective coating layer and the amount of said compound 0.5 to 500 g. per 1 kg. of gelatin in said layer.

9. The silver halide photographic sensitive material as claimed in claim 1, wherein said antifoggant compound is a member selected from the group consisting of methyl-3-(1-aziridinyl)-propionate, 1-(2 - methyl - 1 - aziridinyl)-propionamide, N,N-ethylene-N'-phenyl urea, 1-aziridinyl-propionitrile, 1-acetyl-2-methyl-aziridine, 2-(1-aziridinyl)-4,6 - bis-methoxy-1,3,5-triazine, 1-benzoyl-aziridine, 2-(1-aziridinyl)-4-anilino-6-phenoxy-1,3,5 - triazine, 1-(p-tolyl-

## 14

sulfonyl)-aziridine, 1-phenethyl-aziridine, N,N-ethylene-N'-cyclohexyl urea and 2 - (1 - aziridinyl) - 4,6 - bis-ethylamino-1,3,5-triazine.

10. The silver halide photographic sensitive material as claimed in claim 9, wherein said silver halide emulsion is a silver iodobromide gelatin emulsion.

## References Cited

## UNITED STATES PATENTS

10 2,983,611 5/1961 Allen et al. ----- 96—109 X  
3,128,186 4/1964 Corben et al. ----- 96—109

NORMAN G. TORCHIN, Primary Examiner

15 R. E. FICHTER, Assistant Examiner

U.S. Cl. X.R.

96—107